

# UNITED STATES PATENT OFFICE.

WILLIAM H. SHARP, OF PHILADELPHIA, PENNSYLVANIA.

## MANUFACTURE OF PURIFIED SODA-PINE PULP.

No. 841,190.

Specification of Letters Patent.

Patented Jan. 15, 1907.

Application filed November 8, 1906. Serial No. 342,172.

*To all whom it may concern:*

Be it known that I, WILLIAM H. SHARP, residing at No. 1813 Chestnut street, in the city of Philadelphia, county of Philadelphia, and State of Pennsylvania, have invented a certain new and useful Improvement in the Manufacture of Purified Soda - Pine Pulp, whereof the following is a specification.

As indicated in the above statement, my process is limited to the manufacture of the pulp or cellulose from pine-wood as distinguished from other kinds of wood, and it is also limited to the so-called "soda" process, whereby the wood is primarily digested.

Without attempting to indicate all the varieties of pine whose similar characteristics render them amenable to treatment by my process, the following may be stated as typical of such varieties, the commercial name in each instance being stated as most obviously descriptive—viz., short-leaf spruce-pine, loblolly-pine, foxtail - pine, long-leaf pine, old-field pine, jack-pine, nigger-pine.

When the soda process is employed upon pine-wood of this character, it is found that at the conclusion of the process there are residual substances which resist the purifying reagents and which discolor the pulp, to the serious impairment of its commercial value. These substances do not yield to the bleaching agent usually employed—viz., ordinary bleaching-powder or chlorid of lime—but are extremely persistent; and the object of my present invention is to remove or modify the substances so that they shall no longer impair the product. To this end I conduct the process as follows: The pine-wood in the form of chips or small fragments is first digested

with a solution of caustic soda of the strength of about 12° to 13° Baumé for about ten hours at a pressure of about one hundred and twenty pounds. It is then thoroughly washed with water, and after washing it is treated with bleaching-powder of chlorid of lime, about twenty pounds of this reagent being used to each one hundred pounds of the washed pulp. After the action of the bleaching-powder is nearly exhausted I add about five pounds of a permanganate salt, preferably permanganate of potash or permanganate of soda, to one ton of the pulp. The mass is then stirred

thoroughly, and as soon as the color indicates that the desired reactions are obtained it is washed with a dilute solution of sulfurous acid until all the soluble traces of the manganeseous compounds have been removed. The pulp is then ready for use in the ordinary manner.

Having thus described my invention, I wish it to be understood that I do not claim, broadly, the use of a permanganate in connection with the bleaching of pulp, for I am aware that in the so-called "sulfite" process for the manufacture of pulp permanganate has been used. Its use, however, so far as I am aware, has been at a different stage of the process and in greatly larger percentages than the one which I employ. The soda process, to which my invention is limited, presents entirely different conditions at that stage in which I employ the permanganate, and although the defective character of the ultimate product of the soda process in the particulars above named has long been known and the desirability of a remedy therefor has been fully appreciated, it has not, so far as I am aware, been deemed possible to obviate the difficulties. I therefore base my claim of novelty upon the discovery that where pine-wood is subjected to treatment by the so-called "soda" process the reactions which occur and the resultant condition of the product which is attained after the usual bleaching stage has been completed are such as to permit the successful use of a relatively small amount of permanganate for removing the last and persistent traces of discoloring material.

I claim—

The hereinbefore-described process of manufacturing soda-pine pulp, which consists in, first, digesting the pine-wood with a caustic soda; second, washing; third, treating with chlorid of lime; fourth, treating with a permanganate; and, finally, washing in a dilute sulfurous acid, substantially as set forth.

In testimony whereof I have hereunto signed my name, at Philadelphia, Pennsylvania, this 5th day of November, 1906.

WILLIAM H. SHARP.

Witnesses:

JAMES H. BELL,  
E. L. FULLERTON